

Nov. 21, 1950

O. H. WAECHTER

2,531,016

TREATMENT OF FIBRO-CEMENT PRODUCTS

Filed Sept. 15, 1945



INVENTOR.  
OTTO H. WAECHTER.

BY

*Otto H. Waechter*

ATTORNEY.

## UNITED STATES PATENT OFFICE

2,531,016

## TREATMENT OF FIBRO-CEMENT PRODUCTS

Otto H. Waechter, North Plainfield, N. J.

Application September 15, 1945, Serial No. 616,529

3 Claims. (Cl. 92—41)

1

This invention relates to the treatment of fibro-cement products such as shingles, sidings, and the like to condition them in respect of their moisture content prior to pressing or texturing. More particularly, the invention relates to the treatment of such products made from laminated asbestos-cement sheet material produced on a wet machine by the well known Hatschek process.

According to the Hatschek process a thin web of an aqueous mixture or slurry of Portland or hydraulic cement and asbestos or other mineral fibers, with or without other ingredients, is formed on the endless belt or blanket of a wet machine of the cylinder or Fourdrinier type. The web is carried by the belt to an accumulator drum or roll whereon it is wound, a number of times, until a laminated material of the desired thickness has been formed. The material is then slit lengthwise of the drum, removed therefrom, and spread or opened out into a flat sheet. The sheet so produced is cut into elements such as shingles, sidings, and the like, which elements are subsequently subjected to a pressing operation to give them a finished textured or plain surface that enhances their appearance.

The pressing operation is performed either by means of a pressure roll or in a hydraulic press under high pressure. Where it is desired to finish the elements with a textured surface, as for example in simulation of wood grain, the periphery of the pressure roll is formed to effect the texturing by contact pressure with a surface of the elements, or the elements are formed into a stack with suitable texture plates interposed between adjacent ones and the stack is pressed to effect the texturing.

The laminated asbestos-cement sheet material, as it is removed from the accumulator drum and cut into elements, has a moisture content usually amounting to from about twenty-two to thirty-five percent by weight. Prior to pressing or texturing the elements this normal moisture content must be substantially reduced because if the moisture content is too high deformation of the product will result in the pressing operation, while if it is too low the product will crack.

It is necessary to effect the pressing while the material is still somewhat plastic and before the cement has fully set. Heretofore it has been the practice to form the elements into stacks, either with or without intervening plates, depending upon whether the pressing or texturing was to be done by a roll or in a press, and to allow them to become partially dry before pressing.

That practice has been unsatisfactory not only

because it is slow and entails additional handling but, more especially, because it does not afford a positive control of the moisture content. It often happens that the elements in the middle portion of the stack retain a somewhat higher moisture content than the others. Non-uniformity of moisture content, particularly in the outer strata of the elements, at the time of pressing or texturing, results in the production of an unduly large number of rejects or seconds.

To obtain the best results it is essential that the moisture content of the elements should be uniform at the time they are pressed. I have found that at that time the moisture content should not be more than from about 15—25% by weight.

The principal object of the invention is to provide a method of conditioning the elements to effect a positive control of their moisture content prior to pressing or texturing.

Another object is to provide a method that requires no handling of the product from the time that the sheets are removed from the accumulator drum until after the blanks have been pressed or textured, and that results in reducing the cost of production.

A further object is to provide a method whereby by pressing or texturing of the product is greatly accelerated and that results in the production of products of uniform quality and appearance.

Further objects and advantages of the invention will be apparent to those skilled in the art from the following description thereof.

The invention will be described with reference to the accompanying drawing which illustrated diagrammatically, in side elevation, a form of apparatus suitable for practicing the process.

A web of asbestos-cement, as formed on a conventional wet machine (not shown), is wound in convolutions or laminations on an accumulator drum or roll 10, disposed above on opposition roll 11, until the material on the accumulator drum has been built-up to the desired thickness. Thereupon it is stripped from the drum, opened out, and deposited on a conveyor 12 which carries it under a rotary cutter 13 and over a bed roll 14. The cutter severs the sheet into elements of the desired size and shape.

The elements are carried from the cutter on a conveyor 15 to an endless belt or conveyor 16 which progresses them through an elongated heating chamber 17 wherein they are conditioned by application of heat of a temperature above ordinary room temperature for a sufficient length of time to reduce their moisture content to about

from fifteen to twenty-five percent by weight. The conveyor 16 may operate continuously or intermittently. The chamber 17 may be heated by gas burners 18, electricity, radiant heat, or in any other suitable manner.

An important feature of the process consists in reducing the moisture content in the outer strata of the laminated elements uniformly prior to the application of pressure. In the conditioning step of the process temperature and time are correlative factors, that is the time or rate of progress of the elements through the heating chamber may be shortened if the temperature is raised, or it may be lengthened if the temperature is decreased. The absolute degree of temperature used is unimportant.

On leaving the heating or conditioning chamber, the elements may be carried by the conveyor 16 through a cooling section 19 where they are somewhat cooled by exposure to the air.

The elements then pass to a conveyor 20 that carries them under a pressure roll 21 and over an opposition roll 22. The face of the pressure roll 21 may be formed with a desired texture design, such as wood grain, stonework, etc., either in intaglio or relief, so as to impress or emboss the design on the surface of the elements. Instead of using a pressure roll any suitable press may be employed. Reduction of the moisture content results in a partial hardening of the elements to such a degree that they may be pressed without the excessive elongation or deformation that would occur if the blanks were not properly conditioned.

The pressed elements are delivered by a conveyor 23 and may then be trimmed, if necessary, packed in bundles or stacks and allowed to set and cure in the usual manner.

The process is continuous in the sense that no handling of the product is required from the time that the sheets have been stripped from the accumulator drum until after they have been conditioned and pressed. Moreover, the process is subject to definite control as to uniformity in the quality of production. In practice of the process, should it be found after the first element has been pressed that it had not been properly conditioned as to its moisture content, the temperature and/or time factors can easily be controlled to insure proper conditioning and uniformity of quality throughout the entire subsequent run.

What I claim is:

1. A process of treating asbestos-cement products which consists in continuously and suc- 55

sively progressing a series of cut freshly formed laminated asbestos-cement sheets having a moisture content of from about 22% to 35% by weight first through a heating zone to condition the sheets for pressing by heating said sheets sufficiently to reduce the moisture content from the outer laminations to about 15% by weight, then through a cooling zone of room temperature, and finally subjecting the cooled moisture conditioned sheets to pressure to form a densified asbestos-cement product.

2. A process of treating asbestos-cement products which consists in continuously and successively progressing a series of freshly formed laminated asbestos-cement sheets having a moisture content of from about 22% to 35% by weight first through a heating zone to condition the sheets for pressing by heating said sheets sufficiently to reduce the moisture content from the outer laminations to about 15% by weight, then through a cooling zone of room temperature, and finally subjecting the cooled moisture conditioned sheets to rolling contact pressure to form a densified asbestos-cement product.

3. A process of treating asbestos-cement products which consists in continuously and successively progressing a series of freshly formed laminated asbestos-cement sheets having a moisture content of from about 22% to 35% by weight first through a heating zone to condition the sheets for pressing by heating said sheets sufficiently to reduce uniformly the moisture content from the outer laminations to about 15% by weight, then through a zone of room temperature, and finally subjecting the moisture conditioned sheets to pressure to form a densified asbestos-cement product.

OTTO H. WAECHTER.

#### REFERENCES CITED

The following references are of record in the file of this patent:

#### UNITED STATES PATENTS

| Number    | Name           | Date           |
|-----------|----------------|----------------|
| 1,332,457 | Burkhardt      | Mar. 2, 1920   |
| 1,785,357 | Levin          | Dec. 16, 1930  |
| 1,927,047 | Robinson       | Sept. 19, 1933 |
| 2,006,392 | Greider et al. | July 2, 1935   |
| 2,348,804 | Gerity         | May 16, 1944   |

#### FOREIGN PATENTS

| Number  | Country       | Date         |
|---------|---------------|--------------|
| 354,001 | Great Britain | Aug. 6, 1931 |